

H. H. FIELD, M. HOWARTH & E. A. ATKINS.  
GALVANIZING WIRE, HOOPS, SHEETS, AND THE LIKE.  
APPLICATION FILED FEB. 11, 1913.

1,133,628.

Patented Mar. 30, 1915.



WITNESSES:

John C. Sanders  
Albert F. Heuman

INVENTORS:

Henry Hatten Field  
Mark Howarth  
Evan Arthur Atkins  
by *John H. Muller, Atty.*

# UNITED STATES PATENT OFFICE.

HENRY HATTEN FIELD, OF GRAPPENHALL, MARK HOWARTH, OF LATCHFORD, AND  
EVAN ARTHUR ATKINS, OF LIVERPOOL, ENGLAND.

## GALVANIZING WIRE, HOOPS, SHEETS, AND THE LIKE.

1,133,628.

Specification of Letters Patent. Patented Mar. 30, 1915.

Application filed February 11, 1913. Serial No. 747,719.

To all whom it may concern:

Be it known that we, HENRY HATTEN FIELD, MARK HOWARTH, and EVAN ARTHUR ATKINS, subjects of the King of England, residing at Grappenhall, in the county of Chester, England; Latchford, in the county of Chester, England, and Liverpool, in the county of Lancaster, England, respectively, have invented new and useful Improvements in or Connected with Galvanizing Wire, Hoops, Sheets, and the like, of which the following is a specification.

This invention has reference to the covering or coating of iron and steel—wire, bands, strips, sheets, and other forms of articles, with zinc, by what is known as the "galvanizing" process; and it has primarily for its object to provide improvements in connection with the process of hot galvanizing, by which the quantity of "dross" and oxid formed in the process is reduced or eliminated, at the same time this effect is accomplished with very little expense.

In galvanizing iron and steel wire, (or other articles) by the ordinary hot process, it is customary for the wire or metal previous to entering the molten metal, to pass through dilute hydrochloric acid. In this way, the acid reacts upon the scale or oxid of iron which generally exists upon the surface of the wire or metal forming iron chlorid in solution, which adheres to the surface of the wire, and is carried into the molten metal. The solution of iron chlorid on the wire, meeting the molten zinc, is decomposed into its constituent elements, iron and chlorin; the iron combining with the zinc forming "dross" which falls to the bottom of the bath; the chlorin, at the same time combining with the zinc forming zinc chlorid. The zinc chlorid formed by these reactions, we find, is the flux that actively assists the wire or other iron or steel article to galvanize, by obviating the formation of iron oxid or decomposing any iron oxid that may be on the surface of the article; the zinc chlorid combining with the oxygen, forming oxy-zinc chlorid; the iron being liberated unites with zinc again forming "dross." Some of the water of solution which is carried by the article into the bath, is also decomposed by the molten metal, thus freezing oxygen and forming oxid of zinc. Upon these reactions, the invention hereunder is based and applied to the ends and effects

hereinafter described. This latter chemical reaction also takes place in the ordinary process of sheet galvanizing, in which it is customary to employ ammonium chlorid as a flux; zinc chlorid being here again the real reducing agent. In the same way, other fluxes are used in the galvanizing process to effect the same purposes. In the cases of the use of all these fluxes, the chemical reaction taking place, causes the liberation of iron, chlorin, and oxygen, which instantly combine with the molten metal, forming "dross", oxid, et cetera, in the manner described. In and by the present process, the employment of fluxes is rendered more easy.

In the present process, the prevention of the formation of "dross" is effected by, prior to the iron or steel article being subjected to the action of the molten metal, removing the chlorid and oxid of iron from its surface, and also preventing any oxid forming on it after its removal, and before it reaches the molten metal; and this is effected by an electrolytic action upon it in a bath or vessel containing a suitable electrolyte, such as hereinafter specified, through which the iron or steel article is passed prior to passing into the molten zinc metal, which has the combined effect of removing the oxid from the iron or steel article as stated, and also of depositing a protective covering on it, so that the formation of oxid on it, after it leaves this electrolytic treatment, and before it enters the molten metal, is prevented. By this treatment or process, when the iron or steel wire or other article, enters the bath of molten zinc metal, it carries no free iron compounds in solution, or iron oxid on its surface, and therefore, the chemical action due to these, when brought into contact with the molten zinc metal, is obviated; and in this way the process avoids any exchange of iron compounds with the zinc metal, and so in this manner, the primary object of the invention is accomplished, namely, the saving of waste or loss in the form of "dross", oxid, and the like, as no reducing action, resulting in the liberation of free iron takes place; while also, and due to the same causes, little or no free oxygen is liberated. In addition to the above advantages, others, in respect to the mechanical characteristics connected with the carrying out of the process of hot galvanizing, are rendered possible by the non-production of "dross" in the

process; as for instance, the substitution of bottom or internal heating for side heating, which is much more effective and economical than the latter method. The life of the bath 5 or pot containing the molten metal, will also be considerably increased; and on account of the prevention of the chemical reactions which take place on the surface of the molten zinc, there will be a considerable reduction in the volume of fumes that pass off 10 into the atmosphere.

The wire or metal to be treated will be pickled, as usual; and after pickling, may be washed, immediately before it is moved 15 into the electrolytic apparatus, so that on entering this apparatus and being subjected to the electrolytic action, it will have upon its surface, either the pickling liquid, or water.

20 The covering of zinc, electrolytically deposited upon the wire or article, need be only a very thin film, and it is obtained by passing it through a vessel containing a suitable electrolyte, as above described, disposed in the front of the bath of molten zinc metal; and from its passage through this electrolyte, the wire or other article receives a metallic coat of zinc, by the ordinary electrolytic process or action.

25 Any suitable metallic solution may be used as the electrolyte, but that preferred is one in which either zinc chlorid, or stannous chlorid, is the base.

By the wire or metal passing through the 30 acid bath, immediately before entering the electrolytic bath, it would be coated with a solution of iron chlorid, and this iron chlorid is immediately decomposed by electrolytic action and by interchange with the elements 40 in the electrolytic bath forms zinc chlorid and free iron as iron hydrate, and it is covered with a thin coating or film of zinc, and protected.

An arrangement of plant for galvanizing 45 wire strip, or other continuous form of metal, is illustrated diagrammatically in the accompanying drawing.

In the drawing *a* is the wire or other continuous kind of metal; *b* is the acid bath through which the metal is first passed; *c* is 50 the electrolytic cell, containing the zinc chlorid base, *c<sup>1</sup>* being the anode; and *d* the galvanizing bath containing the molten zinc or spelter.

What we claim is:—

1. In galvanizing steel or iron wire, strips, bands, sheets and the like, the process consisting of converting oxid of iron on its surface, to chlorid of iron, by subjecting it to the action of dilute hydrochloric acid; then 60 removing the chlorid of iron so formed by subjecting its surface to an electrolytic action, by passing it through an electrolytic bath of chlorid of zinc, and also simultaneously thereby coating its surface with a thin 65 coating of zinc, by electrolytic deposition; and finally immersing this iron chlorid free and zinc coated iron or steel article in molten zinc; substantially as described.

2. In galvanizing steel or iron wire, strips, bands, sheets and the like, the process consisting of converting the oxid of iron on its surface to chlorid of iron by subjecting it to the action of dilute hydrochloric acid; then 70 removing the chlorid of iron so formed, by subjecting its surface to an electrolytic action, by passing it through an electrolytic bath of chlorid of zinc, the anode of which is a plate or body of zinc, and the article to be coated is the cathode, and also simultaneously 75 thereby coating its surface with a thin covering of zinc by electrolytic deposition; and finally immersing this iron chlorid free and zinc coated iron or steel article in molten zinc, substantially as described.

80 In testimony whereof we have signed our names to this specification in the presence of two subscribing witnesses.

HENRY HATTEN FIELD.

MARK HOWARTH.

EVAN ARTHUR ATKINS.

Witnesses:

MARK FIELD,

SIDNEY FIELD.